

1

3,356,444  
**VARYING-TONE COLOUR EFFECTS IN  
SYNTHETIC FIBRE FABRICS**

Derek Haworth, Upper Cwmbran, Anil Chandrakant Parikh, Caerleon, and John Charles Turner, Ponfhir, England, assignors to British Nylon Spinners Limited, Pontypool, England

No Drawing. Filed Feb. 13, 1964, Ser. No. 344,536  
Claims priority, application Great Britain, Feb. 21, 1963, 6,949/63  
2 Claims. (Cl. 8—21)

## ABSTRACT OF THE DISCLOSURE

There is provided a dyed synthetic nylon fabric exhibiting varying tone colour effects. The fabric is produced from a combination of yarns having at least two different cross-sectional shapes and each of the cross-sectional shapes having different proportions of titanium dioxide therein.

The present invention concerns improvements in or relating to varying-tone colour effects in synthetic fibre fabrics.

The colouring of fabrics can be effected either by dyeing the yarns or fibres from which they are made or by dyeing lengths of the fabric itself. The latter method is called piece dyeing; and it is the usual method employed when plain colours are acceptable, as in plain tufted carpet material.

Notwithstanding that piece dyeing is primarily a single colour process, it is known that pattern effects in piece-dyed fabrics can be created by the use of yarns which either accept colour differently from one another, by reason of having differing dye uptakes, or by reason of a chemical dye-resist treatment having been applied to only some of the yarns, or which appear different in tone after dyeing by reason of the differing light reflecting properties of the yarns used.

In our British patent specification No. 854,335 we have described how to produce such pattern effects in piece-dyed carpet fabrics by employing some nylon yarns the fibres of which had been heat-set as fibres and other nylon yarns the fibres of which had not been heat-set until spun into yarns.

So far as nylon yarns and fibres are concerned, other methods of producing pattern effects in piece-dyed fabrics are resist processes in which, for instance, the amine ends of the nylon polymer chain are blocked in some of the yarns, and differential orientation processes in which some of the filaments are drawn to a different degree from the others.

The above instanced resist process, however, limits the dyeing process to the use of anionic dyes. Effectively, too, the differential orientation processes are limited to the use of sensitive kinds of dyestuffs, such as certain acid and pre-metallised dyestuffs which are sensitive to rate of dyeing differences between yarns, which will tend to exaggerate any extraneous non-uniformities in the yarn.

We have now found a way of producing varying-tone colour effects in piece-dyed synthetic fibre fabrics, especially nylon fabrics, which enables distinctive tones to be produced without necessary limitation to the use of dyestuffs of a special or critical nature.

According to the invention, a dyed, synthetic fibre fabric exhibiting varying-tone colour effects contains a yarn or yarns composed of synthetic fibres and/or filaments, some of the said fibres or filaments differing both as to their cross-sectional shape and their delustrant content from the others.

2

The yarns can be wholly of short, staple length fibres or wholly of filaments, or some of the yarns can be of such fibres and some of filaments. Alternatively, some or all of the yarns can be of both fibres and filaments, for instance of plied or core-spun type. Unless the contrary is clear from the context of its use, the term "fibres" used herein includes filaments.

In one form of the invention, two-tone colour effects are employed to produce a visible pattern in the surface of the fabric, by using yarns of one type in selected areas of the surface of the fabric and yarns of another type in the remainder of its surface.

The invention will now be described with particular reference to nylon pile fabrics of two-tone colour effects.

15 The pile fabrics may be carpet fabrics of the type produced on so-called "tufting" machinery; and the yarns used may be bulked continuous filament yarns.

Two ends of such yarn, each of polyhexamethylene adipamide continuous filaments and totalling some 3650 20 denier, are creelled alternately. One end of yarn is composed of so-called "quarter dull" filaments of tri-lobose cross-sectional shape; and the other end is composed of so-called "bright" filaments of elliptical cross-sectional shape. The "quarter dull" filaments have a titanium dioxide content of 0.2% by weight, and the "bright" filaments one of 0.03% by weight. The "bright" elliptical cross-section filaments appear darker after dyeing than the "quarter dull" tri-lobose cross-section filaments; and disperse type dyestuffs can be employed with satisfactorily 25 distinctive results.

One end of yarn is tufted with a higher pile than the other in those areas where its colour tone is the one which is required to be visible on the surface.

Instead of an elliptical cross-sectional shape, a circular 30 cross-section is acceptable for the darker-toned filaments.

It is only with the combination of differing cross-sectional shape and differing de-lustrant content that an adequate two-tone effect can be produced. For extra effect, it is of course, often desirable also to modify the dye 35 receptivity of one lot of fibres by a chemical dye-resist process or by increasing the number of basic dye sites available, or to use yarns with different extents of orientation (i.e. yarns the fibres of which have been drawn to different extents), and then use suitable dyestuffs to dye 40 the fabric.

We have referred to a varying-tone colour effect, because the hue is not ordinarily affected according to the invention. The difference in tone may be due either to a difference in dye uptake or to a difference in the light-reflecting properties of the yarns, or to a combination of 45 the two.

Whilst carpet fabric has been exemplified above, it is to be stressed that the dyed fabric may be of any structure, 50 such as a woven or a knitted structure; and the varying-tone effect need not be in patterned areas, but may instead be, for instance, a two-tone effect in some or all of the yarns of the fabric.

We claim:

60 1. A dyed synthetic nylon fabric exhibiting varying tone colour effects, said fabric containing yarns of at least two different cross-sectional shapes selected from tri-lobose, elliptical and circular, and each of the yarn of different cross-sectional shape containing titanium dioxide in different proportions.

65 2. A dyed, synthetic fibre fabric exhibiting varying tone colour effects said fabric containing a first yarn of continuous filaments of polyhexamethylene adipamide having a titanium dioxide content of 0.2% by weight and 70 having a tri-lobose cross-sectional shape and a second yarn of continuous filaments of polyhexamethylene adipamide

having a titanium dioxide content of 0.03% by weight and having a circular cross-sectional shape.

**References Cited****UNITED STATES PATENTS**

2,278,888 4/1942 Lewis ----- 8-14 X  
3,033,240 5/1962 Bottorf ----- 57-140 XR  
3,282,886 11/1966 Gadecki ----- 8-55 X

**OTHER REFERENCES**

R. W. Moncrieff, *Man-Made Fibres*, 4th ed., 1963, pp. 609-610.  
H. C. Speel, *Textile Chemicals and Auxiliaries*, 2nd ed., 5 1957, p. 131.

NORMAN G. TORCHIN, *Primary Examiner*.  
T. J. HERBERT, JR., *Assistant Examiner*.